

# UNITED STATES PATENT OFFICE.

MAX BECKE, OF WEIDLING, NEAR VIENNA, AND WILHELM SUIDA, OF MÖDLING, NEAR VIENNA, AUSTRIA-HUNGARY, ASSIGNORS TO FARBWERKE VORM. MEISTER LUCIUS & BRÜNING, OF HÖCHST-ON-THE-MAIN, GERMANY, A CORPORATION OF GERMANY.

## BROWN DYESTUFFS FOR DYEING WOOL.

1,196,422.

Specification of Letters Patent. Patented Aug. 29, 1916.

No Drawing.

Application filed July 8, 1916. Serial No. 108,219.

To all whom it may concern:

Be it known that we, MAX BECKE, engineer-chemist, and WILHELM SUIDA, Ph. D., professor of chemistry, citizens of the Empires of Germany and Austria-Hungary, respectively, residing at Weidling, near Vienna, and Mödling, near Vienna, respectively, Austria-Hungary, have invented certain new and useful Improvements in Brown Dyestuffs for Dyeing Wool, of which the following is a specification.

We have found that valuable brown dyestuffs for dyeing wool are obtained by subjecting benzoquinone or a halogen derivative thereof to reaction with *p*-phenylenediamin-sulfonic acid. By this reaction the monovalent atomic complex:—



20 enters twice the molecule of the quinone so that compounds are produced which contain the atomic group:



The new dyestuffs are dark-brown powders which are readily soluble in warm water and give on wool brown dyeings of great 30 fastness to washing and to the light, which fastness is increased by subsequently treating them with chromates or copper salts. The process for preparing these dyestuffs consists in heating benzoquinone or a halogen derivative thereof in presence of water with *p*-phenylenediamin-sulfonic acid, or in grinding in a dry state for a considerable time. It is advantageous when using benzoquinone to add an oxidizing agent such as 35 sodium bichromate, and when using chloranil an acid-binding agent.

The following example illustrates our invention, the parts being by weight: 123 parts of chloranil, 188 parts of 1-4-diaminobenzene-sulfonic acid and 272 parts of crystallized sodium acetate are intimately ground for about 24 hours. Thus a blackish-brown 45 product is obtained which readily dissolves in water heated to 70-80° C. to a brown solution which dyes wool in an acid bath a 50 beautiful brown tint, which tint is decidedly

superior, as regards fastness to washing and light and to the action of alkalis to the mixtures of yellow, red and blue acid-dyestuffs hitherto used for the same purposes. When 55 the dyeing is subsequently treated with a chromate or a copper salt, the tint is rendered more intense and its fastness still improved. On precipitating the solution of the product prepared with hot water by means 60 of a mineral acid and salt, the dyestuff may also be obtained in a more concentrated form by filtering the precipitated mixture when cold and drying at a low temperature. A body of similar tintorial properties is 65 obtained by grinding 54 parts of benzoquinone, 188 parts of 1-4-diaminobenzene-sulfonic acid, 98 parts of sodium bichromate and 95 parts of crystallized sodium carbonate.

Having now described our invention, what 70 we claim is:—

1. As new products, the dyestuffs containing the atomic group:



being dark-brown powders, readily soluble in warm water, the solution of which dyes 80 wool tints of great fastness to washing and to the light, this fastness being still improved by subsequently treating with a chromate or a copper salt.

2. As a new product, the dyestuff having 85 the constitutional formula:—



being a dark-brown powder, readily soluble 90 in warm water, the solution of which dyes wool a tint of great fastness to washing and to the light, this fastness being still improved by subsequently treating with a chromate or a copper salt.

In testimony whereof, we affix our signatures in presence of two witnesses.

MAX BECKE.

WILHELM SUIDA.

Witnesses:

AUGUST FUGGER,  
JOHANN FLEISCHMANN.